

April 30, 1940.

H. I. WATERMAN ET AL

2,198,927

PROCESS FOR THE FABRICATION OF EXTRUSION PRODUCTS FROM  
POLYMERIZATION PRODUCTS OF DIENE HYDROCARBONS

Filed March 19, 1938



Inventors: Hein Israel Waterman  
Willem Leendert Johannes de Nie

By their Attorney: L. J. O.

## UNITED STATES PATENT OFFICE

2,198,927

## PROCESS FOR THE FABRICATION OF EXTRUSION PRODUCTS FROM POLYMERIZATION PRODUCTS OF DIENE HYDROCARBONS

Hein Israel Waterman and Willem Leendert Johannes de Nie, Delft, Netherlands, assignors to Shell Development Company, San Francisco, Calif., a corporation of Delaware

Application March 19, 1938, Serial No. 197,632  
In the Netherlands May 8, 1937

8 Claims. (Cl. 18—54)

The present invention relates to a new and improved process for the fabrication, from polymerization products of diene hydrocarbons, of continuous, non-supported objects of small cross-section such as films, ribbons, threads, fibers, foils and the like, which objects, since they are formed by the extrusion of a solution of a polymerized diene hydrocarbon through a suitable die, orifice or nozzle, we designate as "extrusion products." The invention especially relates to a new and improved process for the fabrication of useful threads from polymerization products of butadiene.

It has long been known that synthetic fibers could be made from the polymerization products of diene hydrocarbons, such as butadiene and isoprene. The products fabricated, however, have until recently been of such inferior quality that little importance was ascribed to the process for their fabrication. The threads were thick, dark-colored, non-uniform, either brittle and hard or low-melting and easily extensible, of very low tensile strength and were very difficult to fabricate. Recently, however, improvements have been made which have eliminated many of these faults. These improvements may be divided into two categories, namely, improvements concerning the preparation of the spinning solution and improvements concerning the fabrication of the filament.

While the effect of various co-polymers, impurities, solvents, catalysts, and methods of polymerizing have far-reaching influence on the properties of the finished product, it has been found that its properties are no less dependent upon variations in the methods for forming and treating the viscous thread.

The accepted methods for the fabrication of threads from polymerized diene hydrocarbons consist essentially in spinning the molten polymer, or solution thereof, into a long, vertical, heated tube wherein the solvent, if present, is vaporized and the polymer filament given sufficient heat treatment to render it strong enough for subsequent handling and further hardening.

This method of fabricating has certain inherent defects which result in a thread of impaired strength, color, etc. The method requires high spinning speeds in order to avoid the continual breaking of the thread at the orifice. This is due to the fact that the polymer solution at the spinning nozzle, even when no solvent is present, is in reality nothing more than a thick, viscous liquid in the form of a thread which cannot support its own weight when stationary. In

order to produce a thread of sufficient strength to withstand subsequent processing, this thread must undergo considerable hardening. Since the fast spinning rate necessarily employed allows only a very short time, this necessitates drastic conditions of hardening, such as temperatures ranging from 200° C. to over 500° C., depending upon the diameter of the thread. Such drastic conditions not only tend to discolor the thread, but tend to overharden the outside portion of the thread which in turn impairs the strength and by hindering the diffusion of the solvent contained in the center of the thread makes a longer or more drastic final hardening treatment necessary, and may give a false flexibility. A "false flexibility" due to small amounts of volatile constituents remaining in the center of the filament, results in an early aging and embrittlement of the filament caused by the slow diffusion of the plasticizing solvent. This difficulty cannot be overcome by increasing the length of the heated tube, since this increases the weight of the suspended thread which in turn requires a greater spinning speed in order to avoid parting of the thread near the spinning orifice. Further, in order that the thread shall have sufficient strength at the spinning nozzle, it is customary to spin concentrated solutions of the polymer. This has the disadvantages of requiring high spinning pressures, and also, since there is less shrinkage, of requiring orifices of smaller diameter to produce a thread of a given denier. The small orifices, in turn, require higher spinning pressures, clog more easily and are more costly. The method is furthermore not applicable to the production of objects of other than circular cross-section, since flat objects tend to curl, thicken and warp under the severe conditions.

It is an object of the present invention to provide a method for the production of threads from the polymerization products of diene hydrocarbons, which allows the threads to be spun from dilute solutions of the polymer.

A further object of the invention is to provide a method for the production of threads from the polymerization products of diene hydrocarbons which avoids such heat treatment as may cause discoloration and weakening of the threads.

Still a further object of the present invention is to provide a method for the production of stronger threads from the polymerization products of diene hydrocarbons.

It is also within the contemplation of the invention to provide a method for the production of other continuous, non-supported objects of

small cross-section, such as foils, ribbons, films, etc., from the polymerization products of diene hydrocarbons.

It is also an object of the invention to provide a method which is economical and applicable on a commercial scale.

Other objects and advantages of the invention will become apparent from the following description.

10 These objects, we have found, may be realized by employing a suitable "wet spinning process," followed by a preliminary hardening process.

Although "wet spinning" methods have been employed for the production of other types of 15 synthetic threads, it could not easily be foreseen that such methods would be applicable to the production of the present threads, and, furthermore, are not without considerable modification. This is due to the inherently different characteristics

20 of the present coagulated threads. Unlike the freshly coagulated viscose threads, for example, the present threads are coagulated by diffusion of the solvent portion and not by chemical reaction. This necessarily requires a much 25 longer time. Furthermore, the threads, even when completely coagulated, are exceedingly tender and sticky, and therefore require special methods of handling. For example, the tensile strength of the filament is usually in the order 30 of 0.2 gm. per filament and rarely exceeds 1.0 gm. per filament even in filaments of high denier number. These coagulated threads, whether spun "dry" according to accepted methods or spun "wet" according to the present invention, 35 only become strong and non-sticky after a suitable hardening treatment.

According to the method of the present invention, a suitable solution containing a polymerized diene hydrocarbon is spun vertically through an 40 orifice into a suitable coagulating liquid, wherein a portion of the solvent diffuses from the thread into the liquid. The partially coagulated thread is then subjected to a further coagulating and preliminary hardening treatment. This 45 may be accomplished in either one of two ways. According to the first method, the partially coagulated thread is wound on suitable cylinders or drums rotating with the lower portion submerged in a coagulating liquid. After rotating 50 for several hours, during which the thread is continually wet with the coagulating liquid, the thread is completely coagulated and ready for the preliminary hardening treatment. This is accomplished by rewinding the thread from the 55 cylinder onto reels and allowing to stand for a few hours in air at room temperature and then for 24 hours at a temperature of about 32° C. The thread after this treatment is non-sticky and ready for the final hardening treatment.

60 The above method of completing the coagulation and preliminary hardening, due to the fragility and stickiness of the partially coagulated thread, is beset with numerous mechanical difficulties, and, moreover, is quite lengthy. For 65 these reasons we prefer the second alternative method. According to this second method, we subject the partially or completely coagulated thread issuing from the coagulating bath to any 70 final coagulating treatment necessary and a preliminary hardening treatment in one operation. This is accomplished by passing the coagulated or partially coagulated thread into a bath of hot liquid, such as glycerine. The thread, after this treatment and, if desired, a water wash, is ready 75 for final hardening treatment.

The final hardening may be accomplished by 5 any one of the well-known methods. One suitable method consists in heating the threads for a suitable length of time in an oxygen-free atmosphere. During this treatment, we believe, the polymerization reactions are caused to proceed to the necessary extent to impart the desired qualities of strength and low extensibility.

The present invention is applicable to the fabrication of extrusion products from the polymerization products of any of the diene hydrocarbons capable of yielding products of suitable properties, such as, for example, the polymerization products of butadiene, cyclopentadiene and butadiene substituted in one or more positions by a hydrocarbon radical, for example, isoprene, piperylene, phenylbutadiene and the like.

10 The invention is, furthermore, applicable to the polymers of diene hydrocarbons when these are mixed with or polymerized with other types of polymerizable or partially polymerized substances, for example, vinyl chloride, vinyl bromide, vinyl acetate, chloroprene, natural rubber, cyclocaoutchouc, styrol, compounds of the structure



30 wherein R<sub>1</sub>, R<sub>2</sub>, R<sub>3</sub> and R<sub>4</sub> represent hydrogen atoms and/or organic radicals, and the like. Such polymerized materials are intended to be comprehended by the term "a polymerization product of a diene hydrocarbon." For example, we have found vinyl compounds, such as vinyl acetate, when polymerized with butadiene to impart very desirable characteristics to the products, namely lower extensibility and greater strength. Similarly, other materials may be used to impart special characteristics to the products.

35 The invention is not restricted as to the catalyst used, nor to the mode of polymerizing to 40 form the polymer solution. Suitable catalysts applicable for the purpose include the alkali and alkali earth metals, their mixtures and alloys, peroxides such as benzoyl peroxide, ozonides, such as carvene ozonide, the halides of amphoteric elements, such as SnCl<sub>4</sub>, PCls, etc., as also various other weaker acting polymerization catalysts such as SO<sub>2</sub>Cl<sub>2</sub>, P<sub>2</sub>O<sub>5</sub>, POCl<sub>3</sub>, etc. Of these catalysts, it is found that those of the first class, namely the alkali and alkali earth metals and their mixtures and alloys, are very efficient for the polymerization of diene hydrocarbons and yield products of excellent properties. The other types of catalysts are known to produce polymerization products of different characteristics, and are mainly recommended for the polymerization of diene hydrocarbons with other substances. For example, butadiene and vinyl acetate are best polymerized together with benzoyl peroxide.

45 The polymerization, if desired, may be carried out in the presence of any suitable solvent, or 50 part or all of the solvent may be added after the desired degree of polymerization has taken place. As examples of some applicable solvents may be mentioned the, aromatic hydrocarbons such as benzene, toluene, etc., cycloparaffin hydrocarbons, such as cyclohexane, etc., chlorinated hydrocarbons such as methylene chloride, carbon 55 60 65 70 75 80 85 90 95

5 tetrachloride, ethylene chloride, etc., ethers such as diethyl ether, dioxane, etc. The various solvents may, moreover, be used in conjunction and/or with or without the addition of permissible proportions of non-solvents, such as ketones, alcohols, etc.

10 According to the present invention, unusually dilute solutions of the polymers may be employed. For example, we have found that solutions containing only 10% of dissolved polymer may be conveniently spun according to the present method. This is advantageous since it obviates the concentrating of the polymer solution, facilitates the removal of foreign matter, such as catalyst particles, dust dirt, lint, etc., facilitates the complete homogenizing of the polymer, allows lower spinning pressures and allows the fabrication of threads of low denier number from inexpensive orifices.

15 20 If desired, colored threads may be produced by incorporating a suitable dye prior to the spinning. A suitable dye should, however, be sufficiently heat stable to withstand the subsequent treatments of the thread.

25 The polymer solution is spun vertically into the coagulating liquid by a conventional spinning nozzle. Since the weight of the thread is practically neutralized by the buoyancy of the coagulator, it is not necessary to spin rapidly. The 30 thickness of the thread, the character of the coagulating liquid and the length of path travelled in the coagulating liquid before the thread comes in contact with a solid surface are the factors determining the maximum spinning rate 35 possible.

40 A special embodiment of the process consists in spinning the polymer solutions into a vertically disposed leg of a V-shaped tube filled with a coagulating liquid, and pulling the coagulated thread from the inclined leg. In such an apparatus the rate of spinning is so regulated that the thread is sufficiently coagulated to resist 45 sticking upon passing under suitable guide-rolls placed in the vertex of the V-shaped tube.

50 55 The function of the coagulator is to dissolve the solvent from the spun polymer solution without dissolving the polymer, thus leaving the polymer thread sufficiently strong and non-sticky to be further processed. Consequently, we may use any compound or solution capable of performing this simple function. The coagulator may consist essentially, therefore, of one or more of such compounds as methyl alcohol, ethyl alcohol, isopropyl alcohol, benzyl alcohol, acetone, methyl ethyl ketone, aceto-phenone, butyraldehyde, benzaldehyde, etc. Methyl alcohol, ethyl alcohol and acetone are inexpensive, readily available and, moreover, exceptionally fast acting coagulators, e. g., if benzene is used as a solvent.

60 65 The coagulator liquid, upon becoming sufficiently diluted with solvent extracted from the polymer solution, should be replaced by fresh coagulator liquid. This may be done between runs, but is more conveniently accomplished by continually adding fresh coagulator to the bath and continually withdrawing used coagulator at the same rate. The flow of coagulator thus induced may be either concurrent or countercurrent to the movement of the thread.

70 75 The thread issuing from the coagulator liquid, although sufficiently coagulated to resist sticking upon coming in contact with a surface wet with the coagulator, usually is not coagulated at the center. It is of very low tensile strength, very extensible and prone to become sticky upon dry-

ing. We subject this thread, according to the preferred method of the invention, to a preliminary hardening treatment which consists in heating the thread for a short time in a suitable liquid medium at a temperature above 80° C. and preferably above 100° C. For example, the thread issuing from the coagulator is immediately conducted through a bath of glycerine held at about 140° C. This treatment besides insuring the loss of sticking properties and the complete 10 coagulation of the thread, enhances the tensile strength and lowers the extensibility.

15 The appended drawing illustrates a suitable form of apparatus for executing the process of the invention. The polymer solution enters the 20 spinning nozzle 1 and, in the form of the thread 2, is spun vertically in the coagulating liquid 3 contained in the V-shaped tube 4. The thread is directed around the vertex of the V-shaped tube by means of the guide-rolls 5 and is passed up 25 the inclined leg out of the coagulating liquid. The coagulator liquid is fed continuously into the V-shaped tube through inlet 6 and is withdrawn continuously therefrom through outlet 7. After leaving the coagulating liquid, the thread 30 is passed into a suitable liquid 8 contained in vessel 9 where it is subjected to the preliminary hardening treatment. The liquid in the preliminary hardening bath is heated and maintained at the desired temperature by means of heating 35 coil 10. The thread is pulled out of the preliminary hardening bath and may then be passed to suitable apparatus for the final hardening.

40 Since the purpose of the preliminary hardening treatment is to cause the decrease of the 45 sticking properties and to cause the hardening reactions taking place within the thread to proceed in a controlled manner to produce threads of maximum tensile strength, any heat stable liquid which will not dissolve or attack the thread 50 may be used. One group of compounds which we have found both practical and efficient as bath liquids are the higher boiling organo hydroxy compounds such as, for example, primary or secondary hexyl, heptyl, or octyl alcohol, glycols, glycerine, etc. Lower boiling liquids, such as many of the substances suitable as coagulators, may, however, also be used. These lower boiling liquids, since they involve the use of pressure, are less practical for the continuous 55 treatment, but may find application in a discontinuous method of effecting the preliminary hardening, such as, for instance, by autoclaving.

60 The thread may vary in physical properties, depending upon the time and temperature of the 65 preliminary hardening treatment. Upon subjecting the thread to a prolonged preliminary hardening treatment, it is hardly possible to produce threads of sufficient strength, etc., to meet the usual requirements. It is, however, usually more convenient to effect the final strengthening of the thread by a conventional final hardening process, and this method generally gives a thread with good properties. Thus, we may effect a 70 moderate degree of hardening according to our preliminary hardening treatment, and finally develop the maximum strength in the thread by a conventional final hardening treatment.

75 A special embodiment of our process, according to which the difficulties which are generally encountered owing to the stickiness to which the coagulated thread tends, as soon as it is no longer surrounded by coagulating liquid, consists in that the solution of polymerized diene hydrocarbon is spun into a suitable coagulating liquid which is 80

heated to a temperature exceeding about 100° C., a suitable temperature being, for example, about 140° C. The resulting coagulated thread, after leaving the hot coagulating liquid, does not or practically not possess the troublesome property of being sticky, and may immediately be subjected to the final hardening treatment, no intermediate final coagulating treatment of the thread being necessary.

10. In this special embodiment the hot liquid bath may consist either of a suitable coagulating liquid, e. g., ethyl alcohol, or of a mixture of a coagulating liquid and of a liquid which removes the stickiness of the coagulated thread, such as glycerine.

The threads produced according to the method of our invention are free from discoloration due to overheating, are of the desired strength and low extensibility, and are suitable to be spun and woven by the conventional methods. The fabrics so produced, especially if interspun or interwoven with other filaments such as viscose silk, acetate silk, wool, etc., are textiles of general usefulness. Threads and fabrics composed entirely of the filaments of the present invention, due to their inertness to various chemicals, solvents, etc., and excellent physical properties, are especially adapted for many industrial uses such as, for instance, cable and other electrical apparatus insulation, chemical and solvent resistant clothing, hoods, bags, filter cloths, etc.

Various aspects of the invention are illustrated, but not limited, by the following description of the laboratory fabrication of a butadiene thread and spinning and weaving experiments therewith.

A polymerization product prepared by polymerization of butadiene of 95% purity in an autoclave at a temperature of 15-20° C. in the presence of about 5% metallic sodium was dissolved, after having been worked up, in benzene to a concentration of about 10% and the solution obtained carefully filtered so as to remove undissolved constituents. The clear polymer solution was then spun into the vertically disposed leg of a V-shaped tube having a total length of 175 cm. and filled with ethyl alcohol. The coagulating thread moved downward in the vertically disposed leg of the tube and was drawn up through the inclined leg. The rate at which the thread was drawn from the coagulator bath with slightly greater than the spinning rate thus causing the thread to be stretched somewhat. This operation may also be carried out separately. The spinning rate was adjusted at about 5-10 meters per minute, at which rate the thread was sufficiently coagulated to prevent sticking as it passed under guide-rollers, placed in the vertex of the V-shaped tube. The alcohol was continuously renewed in the reverse direction to that in which the thread moved. The thread issuing from the alcohol bath could be partially hardened in air and the decrease of the sticking properties could be obtained by passing it through hot glycerine. After being given a final hardening treatment these threads had a tensile strength of over 3 kg./mm.<sup>2</sup> and an extensibility of 5-10%.

The thread of 107 denier was readily twined with one filament of viscous silk (175 denier) in a high speed twining machine.

70. Also four threads were intertwined to form a twined yarn which served as a weft for two fabrics. In one fabric the warp consisted of wool-4 filaments of viscose silk-wool-5 filaments of acetate silk-wool. The denier of the two artificial silk warps were approximately 700 and 750 re-

spectively; the denier number of the weft was approximately 450. In weaving the filament the distribution ratio between the upper and under side was 3:1. 35-40% of this fabric consisted of butadiene polymer.

The second fabric was made with a colored warp consisting of red and yellow wool—one filament viscose silk-wool—one filament acetate silk-wool. 70% of this fabric consisted of butadiene polymer.

10. While the present invention is especially concerned with the fabrication of threads from polymerization products of diene hydrocarbons, the invention is likewise applicable to the fabrication of other extrusion products of small cross-section. For example, ribbons, foils and the like may be made, which, since they are non-hygroscopic, unaffected by weather changes, exceptionally impervious to moisture, insoluble in common solvents, not affected by numerous acids and bases, etc., are useful for many purposes.

15. We are aware that numerous details of the process may be varied through a wide range without departing from the principles of the invention, and we, therefore, do not desire our invention 23 to be limited to the specific embodiments herein disclosed except as defined in the appended claims construed as broadly as permissible in view of the prior art.

28. We claim as our invention:

1. A process for the production of synthetic fibers which comprises forcing a solution of a polymerization product of butadiene containing less than 20% polymer through a suitable spinning-nozzle vertically into a liquid consisting of at least a substantial proportion of a lower aliphatic alcohol, drawing the coagulated thread from said liquid at a rate exceeding the spinning rate, and immediately passing the coagulated thread through a liquid bath consisting of at least 33 a substantial proportion of an organo-hydroxy compound held at a hardening temperature above about 80° C. whereby a completely coagulated and at least partially hardened fiber is produced which may be further treated. 45

2. A process for the production of extrusion products which comprises forcing a solution of a polymerization product of a diene hydrocarbon through a suitable die, into a liquid which is readily miscible with the solvent used but does not appreciably dissolve the polymer and contacting the coagulated extrusion product with a liquid which is at a hardening temperature above about 80° C. and which will not appreciably dissolve or attack the polymer, whereby a completely coagulated and at least partially hardened product is produced which may be further treated. 55

3. In a process for the production of an extrusion product, the steps comprising forcing a solution of a polymerization product of a diene hydrocarbon through a suitable die, into a liquid which is readily miscible with the solvent used but does not appreciably dissolve the polymer and contacting the coagulated extrusion product with a liquid containing at least a substantial proportion 60 of an organo-hydroxy compound which liquid is at a hardening temperature above about 80° C. 65

4. In a process for the production of an extrusion product, the steps comprising forcing a solution of a polymerization product of a butadiene 70 through a suitable die, into a liquid which is readily miscible with the solvent used but does not appreciably dissolve the polymer and contacting the coagulated extrusion product with a liquid 75 which will not appreciably dissolve or attack the 75